

M. M. MERRITT,  
ELECTROLYTIC METHOD, APPARATUS, AND PRODUCT.  
APPLICATION FILED OCT. 7, 1919.

1,363,186.

Patented Dec. 21, 1920.

3 SHEETS—SHEET 1.



Fig. 1.

Inventor:  
Matthew M. Merritt,  
by Emery Booth, Jerny & Verney  
Atty.

M. M. MERRITT.

ELECTROLYTIC METHOD, APPARATUS, AND PRODUCT.

APPLICATION FILED OCT. 7, 1919.

1,363,186.

Patented Dec. 21, 1920.

3 SHEETS—SHEET 2.

Fig. 3.



Fig. 2.



Inventor:  
Matthew M. Merritt,  
by Emery Booth Janney Verney  
Atlys

M. M. MERRITT.

ELECTROLYTIC METHOD, APPARATUS, AND PRODUCT.

APPLICATION FILED OCT. 7, 1919.

1,363,186.

Patented Dec. 21, 1920.

3 SHEETS—SHEET 3.

*Fig. 6.*



*Fig. 4.*



*Inventor:*

*Matthew M. Merritt,*  
*by Emery Booth Janney & Varney*  
*Attny.*

# UNITED STATES PATENT OFFICE.

MATTHEW M. MERRITT, OF SOUTH MIDDLETON, MASSACHUSETTS.

## ELECTROLYTIC METHOD, APPARATUS, AND PRODUCT.

1,363,186.

Specification of Letters Patent. Patented Dec. 21, 1920.

Original application filed April 15, 1919, Serial No. 290,152. Divided and this application filed October 7, 1919. Serial No. 328,999.

To all whom it may concern:

Be it known that I, MATTHEW M. MERRITT, a citizen of the United States, and a resident of South Middleton, county of Essex, State of Massachusetts, have invented an Improvement in Electrolytic Methods, Apparatus, and Products, of which the following description, in connection with the accompanying drawings, is a specification, like characters on the drawings representing like parts.

This invention pertains to improvements in electrolytic methods, apparatus and products. One of the broader aspects of the invention relates to methods and apparatus for depositing metal electrolytically while the electrolyte flows in a stream past the cathode or cathodes, the anodes preferably being distributed in the stream longitudinally there- 15 of and preferably in comparatively close relationship to the cathode surface or surfaces.

Another aspect of the invention relates to the circulation of the electrolyte in such a 25 way that an opportunity is afforded for the same to "rest" so that hydrogen may have an opportunity to escape from the body of the electrolyte during a period when the electrolyte is not being used actively as an 30 electrolytic agent.

Another aspect of the invention includes the aeration thereof in any suitable way, but preferably by permitting the electrolyte to fall through the air a sufficient distance to 35 accomplish this purpose.

While the most important features of my invention are of general application in the electrolytic art, and are useful in making all electrolytically deposited or coated articles or products, I have elected, without limitation thereto, to disclose the same in connection with the deposit of metal on elongated cathodes in connection with the manufacture of electrolytically coated wire and 40 similar products such as tubes formed by electrolytically depositing metal on elongated cathodes adapted to be removed after electro-deposition, leaving the electrolytically deposited shell to form the tube or 45 pipe. Where my invention is applied to the manufacture of coated wire, tubing or pipe, it preferably includes the passage of the wire or other cathode through the electrolytic bath so that each portion of an elongated 50 flexible cathode may be, if desired, sub-

jected to electrolytic action under substantially constant conditions and for substantially the same length of time.

While many features of my invention are of general application, and may be used for 60 any purpose in connection with the deposition of any metal on any form of cathode, I have elected in this application specifically to describe the same in connection with the electro-deposition of copper on a steel cath- 65 ode, of copper on an aluminum cathode (preferably treated as hereinafter more fully described), and in connection with the electro-deposition of copper on a fusible or otherwise removable cathode, the latter be- 70 ing primarily useful in connection with the formation of tubing.

This application is a division of my co- 75 pending application, Serial No. 290,152, filed April 15, 1919.

The drawings show an illustrative embodiment of a preferred form of apparatus useful in connection with practising my improved process as applied to the manufac- 80 ture of wire, tubing and the like.

Figure 1 is a longitudinal section, partly in elevation, illustrating diagrammatically certain preferred forms of apparatus used in performing certain preferred preliminary steps of my method;

Fig. 2 is a side elevation showing a preferred form of apparatus for use in connection with practising my improved method where applied to the manufacture of wire and tubing, the apparatus disclosed in Fig. 90 2 being that in which the principal electro-deposition takes place, preferably subsequent to suitable treatment, hereinafter described, of the anode material by the apparatus shown in Fig. 1;

Fig. 3 is a plan of the apparatus shown in Fig. 2;

Fig. 4 is a section on the line 4—4 of Fig. 2;

Fig. 5 is a section on the line 5—5 of Fig. 100 2; and

Fig. 6 is a section through a preferred form of apparatus for removing the fusible cathode material from tubing made by my method and apparatus.

I will first describe rather specifically, though without limitation of the broader aspects of my invention, the operation of the apparatus shown in the drawings in connection with the manufacture of copper coated 110

steel wire. Steel, iron or other suitable wire 7, preferably coiled on a drum 8, may be drawn from the drum 8 and initially passed through a cleansing agent, preferably muriatic acid and tin chlorid in the tank 9, the wire thence passing under a stream of water 10 to remove any acid which may cling to the surface thereof, and thence into an alkaline bath, preferably cyanid, in the tank 11. This bath 11 is preferably provided with a suitable anode 12, which may be of copper, a negative connection 13 being made to the wire preferably before entering the bath 11. The wire may be fed at any suitable speed, but is preferably immersed in the cyanid bath 11 for a sufficient length of time to plate the wire with copper so as to protect the steel from the subsequent action of the acid when deposition is carried on in an acid bath as hereinafter described. The current density used in connection with plating in this cyanid bath may be as is usual in copper plating processes. After the wire leaves the cyanid bath 11, it is again washed, preferably by passing through a glass tube 14 into which a stream of water is introduced at 15, this providing a very simple and efficient rinsing medium. The wire, thus plated in the cyanid bath and rinsed, is then passed to the apparatus in which further electro-deposition of metal is rapidly carried on under high current density.

Perhaps the most important feature of my improved apparatus and method, which feature is applicable to all kinds of electro-deposition of all metals on all forms of cathodes, includes the passing of the electrolyte in a stream past the cathode. This stream may conveniently be confined in a trough, which may, if desired, slant in two directions as best shown in Fig. 2, the electrolyte being introduced into the trough at 16 and flowing in opposite directions through the trough or troughs 17, 18 and thence flowing into a reservoir or tank 19. The discharge ends of the troughs are preferably at a sufficient distance above the level of the electrolyte in the tank or reservoir 19 to afford a fall of the electrolyte through the air. The tank or reservoir 19 affords a chance for the escape of hydrogen from the electrolyte and is preferably of sufficient depth to permit settlement of any heavy impurities to the bottom and to permit any lighter impurities, such as hydrogen, to rise to the top, while leaving a middle stratum of comparatively pure electrolyte, from which is drawn the supply of electrolyte to the discharge 16, the circulation preferably being effected by any suitable elevating means, herein shown as a centrifugal pump 20. To increase the conductivity of the electrolyte, and to facilitate the escape of hydrogen bubbles, I preferably provide a steam

coil or other heating agent for heating the electrolyte in the tank 19.

It should be clearly understood that the apparatus illustrated is merely a preferred embodiment of my invention, and that various features thereof and various steps of the method used in connection therewith are useful, whether used in combination with other portions of the apparatus and other steps of the method, or whether used separately in any connection. For instance, while I have shown the trough sloping in two directions, it is obvious that a trough sloping in one direction, or any means or suitable mechanism for producing a flow of the electrolyte, is of use. It is also clear that, while I have shown the flow of electrolyte in connection with the electro-deposition on wire, that the flow of the electrolyte is useful when used in connection with cathodes of any kind, whether individual articles continuously immersed in the flow, or whether individual articles intermittently immersed in the flow. It should also be understood that the preferable aeration of the electrolyte, while preferably provided by the fall of the electrolyte from the end or ends of the trough or troughs, may be effected in other ways, and that the provision of means for permitting the electrolyte to "rest," preferably while heated, may be of use in connection with electrolytic processes differing greatly in other details from those herein described. Similarly, while the various features of my apparatus and steps of my method are peculiarly useful in their co-operative relationship, it should be understood that each may be of use in other connections.

Returning to the specific embodiment of my invention shown in the drawings, the wire 7 preferably passes through the trough or troughs 17, 18 a plurality of times, being passed preferably in a generally helicoidal relationship about a series of preferably independently rotatable sheaves arranged in tiers 21, 22 at opposite ends of the troughs, thus providing a continuous length of wire making up two "runs," each "run" preferably including several passages of the wire. The "runs" correspond to the opposite sides of a helicoid viewed as a whole, and the several passages of the wire making up each "run" correspond to the individual turns making up the sides of the helicoid. The tiers of sheaves 21 and 22 may be conveniently used as negative contacts for conducting the current rendering the wires carried by the sheaves the cathodes of the apparatus.

In order to provide for close proximity of the anode material to the wire, I preferably duplicate the troughs 17, 18, providing corresponding trough or troughs for each "run" of the wire. Thus, as best viewed in

Fig. 3, the "run" 23 coöperates with the double inclined troughs 17, 18, and the "run" 24 of the wire coöperates and passes through the troughs 17', 18' fed by a conduit 16' corresponding to the conduit 16 from the pump 20. The troughs 17, 18 and 17', 18' are preferably, as shown, relatively narrow, or, in any case, preferably provide anode surfaces relatively close to the cathodes. As best viewed in Fig. 5, the anodes 10 may be composed of copper sheets or copper scrap retained behind suitable screens such as the perforated lead sheets 40. Any suitable positive connection may be made with these anodes or with the lead screens before referred to, or with the lead lining of the troughs. It is obvious that, if desired, I 15 may provide any desired number of "runs" by changing the arrangement of sheaves 20 over which the wire is passed, and in such case I may provide a correspondingly increased number of troughs. It is also obvious that the depth of the troughs may be increased or decreased to correspond to an 25 increase or decrease in the number of passages of the wire making up each "run." The troughs may be of any suitable length, but I have found by experiment that troughs sloping in one direction thirty feet long, and 30 having a fall of four inches, are satisfactory, and similarly that a trough sloping in two directions, as shown on the drawings, thirty feet long and having a slope of two inches toward each end thereof, provides a 35 very desirable rate of flow, approximating preferably one hundred and thirty feet per minute.

I have shown in Fig. 4 a cross-section on the line 4—4 of Fig. 2, Fig. 4 being on an 40 enlarged scale and showing details of the troughs and coöperating parts adjacent the center of the apparatus. Where troughs sloping in two directions are used, I may provide suitable separating means for the 45 wires to prevent contact of one against the other, herein shown as glass rollers 25. While I preferably make my process a continuous one, joining one roll of wire to the next, it is sometimes necessary to suspend 50 operations and to pass a new wire through the system by a threading, as distinguished from a drawing, operation. To facilitate this, I have provided mechanism, best shown in Figs. 2 and 5, for dropping the tanks 55 away from their operative position so as to permit ready passage of the wire about the sheaves and through the rollers 25. To facilitate raising and lowering of the tanks, I have shown racks 26, 26 coöperating with 60 pinions 27, 27 mounted on shafts 28, 28 and adapted to be turned by cranks 29, 29 and adapted to be locked against undesired rotation by any suitable mechanism, typified by the dog or pawl 30. The troughs 17 65 and 17' may be guided in their vertical

movement in any suitable way, typified by the guides 31, 31 engaging vertical members of a bridge or framework 32 passing above the troughs and supported or guided at their inner sides by rollers 33. The glass rollers 70 25, hereinbefore described, are preferably suspended in frameworks 34, 34 from the bridge 32, which may conveniently also support the discharge conduits or nozzles 16, 16'. 75

As heretofore stated, the current density utilized in connection with the troughs is preferably much higher than the current density utilized in connection with the cyanide bath 11. The rate of deposit on the 80 various portions of the wire exposed to electrolytic action in the troughs varies in proportion to the length of time that the various parts of the wire have been exposed to electrolytic action, the wire as it first enters 85 the trough after being washed pursuant to the cyanide bath being only slightly covered by the cyanide plating operation, and being of comparatively small cross-section and of comparatively slight electrical conductivity 90 as compared with the cross-section and electrical conductivity after considerable electro-deposition has taken place in the troughs. It may be roughly said that the wire at any 95 given time exposed to electrolytic action in the troughs takes the form of a truncated cone, of which the small end is at the beginning and the large end at the finish. Of course, as the operation is continuous, each portion of the wire being subjected to exactly the same treatment as each other portion, the wire as it leaves the finishing point 100 is of uniform diameter and conductivity.

The power for conducting or drawing the wire through the various operations heretofore described may be applied to the winch 35, about which the wire is passed before passing on to a winding drum 36 which is driven through a clutch adapted to slip to compensate for changes in diameter of the 110 drum as the wire is wound thereon. The winch 35 determines the speed at which the wire passes through the apparatus. 105

Just before the wire goes on to the winch, it is preferably washed by washing apparatus 37. 115

Where the apparatus is used for the deposition of copper on a cathode composed of aluminum wire, the acid bath 9 and the cyanide bath 11 need not be used, but some 120 mechanism should be provided for treating the surface of the aluminum wire to remove the oxid on the surface of the aluminum and preferably to deposit a film of foreign substance to serve as an oxid-excluding medium over the surface of the aluminum, and to provide a surface thereto other than aluminum which will readily take in a satisfactory manner the deposit of copper or other metal during subsequent electro- 125 130

deposition. The oxid-excluding medium is preferably tin, and I may effect the combined deoxidizing and tinning operation by supplying the pipe 15 with a mixture of 5 muriatic acid, water and tin chlorid. To obviate the necessity for too rapid circulation of this liquid, I may provide a sponge on the interior of the tube 14 to absorb and check the flow of the cleansing and coating 10 agent, it being necessary only to supply a sufficient quantity thoroughly to clean and coat the surface of the aluminum wire.

While I have described this preliminary 15 treatment of aluminum prior to electro-deposition in connection with the manufacture of a continuous strand of wire, and while this method is of great utility in this connection, it will be understood that this feature of my invention may be useful in other 20 connections such as the preparation of any object made of aluminum or surfaced with aluminum for electro-deposition. The interposition of the coating of oxid-excluding medium between the aluminum and the 25 copper minimizes that galvanic deterioration of these metals which normally arises where, in the presence of even a trace of moisture, copper and aluminum are permitted to come into contact or even into close 30 proximity.

Where my improved method and apparatus is used in connection with the manufacture of tubing and pipes, a cathode of fusible metal or any other suitable conductive 35 substance, or even a non-conductive substance coated with a conductive substance, is substituted for the initial coil of steel wire on the drum 8. Where this readily fusible or otherwise removable core or cathode is 40 composed of lead or an alloy of tin and lead or the like, it is not essential that any preliminary treatment be given prior to starting of electro-deposition in the flowing electrolyte, but where it is desired to provide a 45 tube having an interior coating of tin, I may pass the cathode through an alkaline bath, corresponding to the cyanid bath 11, in which I electrolytically deposit copper on the surface of the fusible metal cathode prior 50 to the electro-deposition of copper or other metal in an acid bath. The passage of the cathode through the flowing electrolyte may be the same as in the case of coating wire, as hereinbefore described, and after electro-deposition is completed the cathode with the 55 electro-deposited metal thereon may be wound in the form of a helix and placed in a melting furnace, shown in Fig. 6, the entire coil being heated to a point sufficient to melt the readily fusible core, but not sufficient to melt the copper surface, and air pressure being applied at 38 to blow the melted fused core from the interior of the tube. Where the initial deposit of copper 60 on the fusible cathode has been made in a

cyanid bath, as hereinbefore described, the interior surface of the copper is chemically clean at the time when the fusible core is melted out, and the tin or similar content in the fusible core will adhere to the interior 70 surface, thus providing a perfectly smooth and perfectly tinned lining to the tube.

The use of an electrolyte which is flowing during electro-deposition enables me to use 75 a much higher current density than has been possible, while securing satisfactory results, in any electro-depositing process heretofore considered possible. I have secured fine-grained, smooth, ductile, uniform, homogeneous electro-deposits in connection with 80 this method and apparatus while using a current density up to one thousand amperes per square foot of cathode surface. None of the deleterious results of the formation of hydrogen bubbles on the cathode, 85 commonly known as spongy deposit, are present where my apparatus and process is utilized. This is due to rapid liberation of the hydrogen arising from several causes; first, the rapid passage of the electrolyte 90 past the cathode surface; second, the fact that no given portion of the electrolyte is actively used continuously for any considerable length of time; third, the fact that no given portion of the electrolyte acts more 95 than momentarily on any given portion of the cathode surface; fourth, the fact that the electrolyte is given an opportunity to "rest" between the periods of recurrent use of any portion thereof, thus providing a 100 time for liberation of the hydrogen and for settlement of any foreign substance heavier than the electrolyte; fifth, the fact that the reservoir 19 provides an opportunity for a 105 lower stratum in which the impurities can settle, an upper stratum in which the hydrogen can be liberated, and an intermediate stratum comparatively clean from which the supply of electrolyte to the trough or troughs can be drawn; sixth, where the apparatus and method is used in connection 110 with the manufacture of a continuous article, such as specifically described herein, the preferably constant passage of the article through the electrolyte insures the absolute uniform treatment of all portions of the cathode, and if, for any reason, conditions exist in any part of the stream such as the absence of anode surface or irregularity of flow of the electrolyte adjacent 115 the point of introduction of the electrolyte or elsewhere, this accidental or otherwise non-uniform condition will act uniformly upon all parts of the wire as it passes through the apparatus, insuring uniformity of product and insuring minimization of deleterious action on any given part of the wire; seventh, the provision of the relatively large reservoir 19 not only provides for "rest" of the bath, but also per- 120

mits heating of the same for a considerable length of time between intermittent periods of use of any given portion of the bath. The amount of electrolyte actually subject to 5 electrolytic action at any one time may be almost negligible in comparison with the amount of electrolyte in the reservoir.

While I have shown in the drawings and described rather specifically a preferred 10 form of apparatus and a preferred method, it will be understood that major changes involving omission, substitution, reversal or other changes in the apparatus as a whole or in parts thereof, and even changes of similar 15 or greater scope in connection with the method, may be made without departing from the scope of my invention, which is best defined by the following claims.

Claims.

20 1. Electrolytic apparatus comprising means for passing a continuous stream of the electrolyte past the cathode.

25 2. Electrolytic apparatus comprising, in combination, means for passing a continuous stream of the electrolyte past the cathode, and anode surfaces for renewing the ionic supply to said stream.

30 3. Electrolytic apparatus comprising, in combination, means for passing a continuous stream of the electrolyte past the cathode, and anode surfaces for renewing the ionic supply to said stream, said anode surfaces being distributed lengthwise of the stream.

35 4. An electrolytic apparatus comprising, in combination, means for passing a continuous stream of the electrolyte past the cathode, and anode surfaces for renewing the ionic supply to said stream, said anode surfaces being distributed lengthwise of the 40 stream and in relatively close proximity to the cathode surface or surfaces.

45 5. Electrolytic apparatus comprising, in combination, a trough, means for introducing a stream of electrolyte into said trough, a reservoir for receiving the electrolyte passing from said trough, and circulatory means for drawing the electrolyte from said reservoir and returning the same to said trough.

50 6. Electrolytic apparatus comprising, in combination, a trough, means for introducing a stream of electrolyte into said trough, a reservoir for receiving the electrolyte passing from said trough, and circulatory means for drawing the electrolyte from said reservoir and returning the same to said trough, said reservoir containing an amount of electrolyte very substantially greater than the amount contained at any one time in said trough.

60 7. Electrolytic apparatus comprising, in combination, an anode containing conduit and means for supplying electrolyte to said conduit to provide for circulation of the electrolyte through said conduit past the 65 cathode.

8. Electrolytic apparatus comprising, in combination, a trough sloping in two directions, reservoir means for receiving the flow of electrolyte from each end of said trough, and means for introducing a stream of electrolyte to said trough at a point adjacent the highest point of the bottom thereof. 70

9. Electrolytic apparatus comprising, in combination, means for progressively advancing a flexible cathode to provide a plurality of runs, each including several passages of cathode material and a plurality of conduits, one for each of said runs, for confining a stream of flowing electrolyte activated to effect electro-deposition on the cathode material. 75 80

10. Electrolytic apparatus comprising, in combination, cathode supporting means, troughs for confining a stream of electrolyte in proximity to the cathode material and means for raising and lowering said troughs into working or non-working position relative to the cathode material. 85

11. Electrolytic apparatus comprising, in combination, circulating means for circulating the electrolyte in a swift-flowing stream passing the cathode, and means providing an opportunity for "rest" of the electrolyte between recurrent passage thereof to said circulating means. 90 95

12. Electrolytic apparatus comprising, in combination, a trough, a plurality of passages of flexible cathode material passing through said trough, a stream of electrolyte discharging into said trough and means for separating said passages of flexible cathode material adjacent the point of entrance of said stream of electrolyte. 100

13. Apparatus for use in connection with electro-deposition comprising a sloping trough, anode material distributed longitudinally of the trough and means for circulating the electrolyte through the trough. 105

14. Apparatus for use in connection with electro-deposition comprising a sloping trough, anode material distributed longitudinally of the trough, means for circulating the electrolyte through the trough and means for aerating the electrolyte. 110

15. Apparatus for use in connection with electro-deposition comprising a sloping trough, anode material distributed longitudinally of the trough, means for circulating the electrolyte through the trough and means for aerating the electrolyte by passing the same over a fall. 115 120

16. Apparatus for use in connection with electro-deposition comprising a sloping trough, anode material distributed longitudinally of the trough, means for circulating the electrolyte through the trough and cathode retainers at the sides of the trough. 125

17. Apparatus for coating an elongated flexible element comprising, in combination, initial coating means for initially coating 130

- said element with a relatively thin protective film, and other coating means for subsequently electrolytically depositing copper thereon.
- 5 18. Electrolytic apparatus comprising, in combination, a sloping trough and means for supplying a stream of electrolyte thereto at a rate which, in combination with the slope of said trough, provides a flow of the electrolyte at a rate exceeding one hundred feet per minute.
- 10 19. Electrolytic apparatus comprising, in combination, a sloping trough, means for supplying a stream of electrolyte thereto,
- said trough being relatively narrow and having anode material distributed lengthwise thereof.
20. Electrolytic apparatus comprising, in combination, a sloping trough, means for supplying a stream of electrolyte thereto, 20 said trough being relatively narrow and having anode material distributed lengthwise thereof in relatively close proximity to the cathode.

In testimony whereof, I have signed my 25 name to this specification.

MATTHEW M. MERRITT.